

Aug. 29, 1939.

B. JONES

2,171,180

LEAD ALLOY

Filed Feb. 24, 1937



Fig. 4.



Fig. 1.



Fig. 2.



Fig. 3.



Fig. 6.

Fig. 5.



Fig. 7.



INVENTOR  
Brinley Jones  
By Watson, Cott, Morse & Grindle  
ATTYS

## UNITED STATES PATENT OFFICE

2,171,180

## LEAD ALLOY

Brinley Jones, Perivale, England, assignor to  
Goodlass Wall & Lead Industries Limited, Lon-  
don, England

Application February 24, 1937, Serial No. 127,470  
In Great Britain June 4, 1936

7 Claims. (Cl. 207—10)

This invention relates to alloys of lead and tellurium containing copper. In British specification No. 414,606 are described alloys of this nature containing a proportion of from 0.01—0.1% of tellurium and 0.01—0.15% of copper, it being stated that the incorporation of the tellurium and the copper in the alloy conjointly imparts to the alloy a greater resistance to corrosion than an equivalent quantity of either of these elements separately.

Extruded products such as cable sheathings or sometimes pipes are often manufactured on a plant which operates with a die having a bridge core. Here it is necessary to extrude at a temperature high enough for the metal to weld together again beyond the bridge core, and the optimum extrusion temperature from this point of view is relatively high, for example, a temperature as close to the melting point of lead (327° C.) as is practicable. On the other hand, the optimum extrusion temperature of lead-tellurium alloys from the point of view of the grain structure of the extruded product is considerably lower.

I have found that as the proportion of copper present in the alloy is increased, the tendency to develop a coarse grain when extruded at a high temperature is progressively diminished. Useful results are obtained with a copper content as low as 0.03%, but it is preferred to keep the copper content within the range of 0.05—0.1%. Particularly good results are obtained when the copper content is from 0.06—0.07%, as then not only is the alloy proof against development of a coarse structure due to burning if the material should subsequently be welded, but also there is no substantial tendency for the copper to segregate.

When, therefore, the lead-tellurium alloy contains copper, the metal can be extruded at a sufficiently high temperature to avoid weaknesses due to inadequate welding together of the metal beyond the bridge core, but at the same time the product retains a fine grain, which results in it having far superior mechanical properties, and in particular a greatly improved resistance to intercrystalline cracking. Also, provided the copper content is above 0.06%, the metal can be subjected to local welding where desired without the fine grained structure being impaired.

The invention will now be described in further detail with reference to the accompanying drawing, in which

Fig. 1 is a photomicrograph, at a magnification

of five, of an etched cross section of a hot extruded pipe made from an alloy of lead containing 0.05% tellurium but no copper,

Fig. 2 is a similar view, at the same magnification, of a hot extruded pipe made from an alloy of lead containing 0.05 tellurium and 0.067% copper,

Fig. 3 is a diagrammatic sectional view illustrating the segregation which occurs in a casting made from a lead alloy containing 0.05% tellurium and 0.08% copper,

Fig. 4 is a side elevation, partly in section, of a bridge core pipe press,

Fig. 5 is an enlarged sectional view of the bridge core of this press, and

Figs. 6 and 7 show respectively a pipe and a cable sheathing.

When manufacturing extruded products, such as pipes or cable sheathing, from lead alloys, it is generally desirable to extrude the metal at as high a temperature as practicable from considerations of speed and convenience of operation. This is particularly so in the case of a bridge core press, where the metal has to weld together again beyond the die.

In the case of binary alloys of lead and tellurium, it is found that the metal recrystallizes with a fine grain when it is extruded at a relatively low temperature, so that the material has improved mechanical properties as compared with extruded soft lead which recrystallizes with a coarse structure. Binary tellurium-lead alloys cannot however be extruded at the high temperatures customary for ordinary soft lead because under these conditions the cast structure is not completely broken down. A structure such as that shown in Fig. 1 develops, with the result that insufficient ductility is obtained. Consequently it has been necessary to extrude binary lead and tellurium alloys at lower temperatures than those which are ordinarily employed for soft lead. Copper tellurium lead alloys extruded at a high temperature possess a very much finer grain than binary tellurium-lead alloys which have been extruded at the same temperature. This is shown in Fig. 2. The result is that the product has improved mechanical properties, in particular an improved ductility as compared with the product shown in Fig. 1. The critical lower limit of 0.06% copper is not decisive as to the grain size of the metal after extrusion, as it is in the case of welding, and pipes and cable sheathings of reasonably fine grain can be made by hot extrusion from cop-

per-tellurium-lead alloys containing as little as 0.03% copper.

It is preferred to keep the copper content below 0.07%, as otherwise some tendency towards 5 segregation is observed, as may be seen from Fig. 3 where the excess copper is indicated at A, having segregated to the top of the casting. It will be appreciated that this figure is diagrammatic only, the segregated copper being shown, 10 for the sake of clarity, on a greatly enlarged scale. The copper content can however be increased to 0.1% without the effects of segregation becoming serious.

The present invention has particular advantages when applied to the manufacture of pipes 15 on a bridge core press. Such a press is shown in Figs. 4 and 5.

It comprises a container 20 mounted on a hydraulic ram, which is operable to raise the container so that it passes over the lower end of a fixed hollow ram 21, which fits exactly within the container. Across the lower end of the ram 21 extends a removable bridge member 22 carrying an upright core 23.

The container is first lowered and filled with molten metal. It is then raised with the result that a hollow tube 24 of metal is extruded between the core 23 and the co-operating die 25. This constitutes the pipe shown separately in Fig. 6.

With such a press, it is clearly desirable to extrude the metal at as high a temperature as possible, in order to ensure that it welds together properly above the bridge 22 to make a good pipe. As explained above, however, a limit to the temperature of extrusion of binary lead tellurium alloy has been set by reason of the coarse structure which develops in the finished pipe. When however a lead tellurium alloy containing from 0.03-0.1% of copper is used, the pipe may be extruded at a high temperature without a coarse structure resulting. This ensures adequate welding together of the pipe. If the alloy contains above 0.06% copper there is the additional advantage that local welding of the finished pipe is possible without developing a coarse structure in the weld.

It is a difficult matter to determine the temperatures prevailing in the container of the extrusion press and the practice is to estimate them by means of pyrometers inserted into the wall of the container and of the die box. In my experiments the ends of the pyrometers extended to a distance of one inch from the metal, and of course the readings are much lower than the actual temperature of the metal. In one case in which extremely satisfactory extrusion of an alloy containing 0.05% tellurium and 0.067% copper was obtained, the readings were as follows:

|                                                                                                | Degrees<br>centigrade |
|------------------------------------------------------------------------------------------------|-----------------------|
| Temperature of metal in the melting pot, which is charged into the container of the press----- | 375                   |
| Temperature indicated by the pyrometer at the top of the container-----                        | 100                   |
| Temperature indicated by the pyrometer at the bottom of the container-----                     | 100                   |
| Temperature indicated by the pyrometer in the die box-----                                     | 150-160               |

The alloys referred to may also usefully be employed for making cable sheathing, a sample

of which is illustrated in Fig. 7. The electric conductor 30 is covered with insulation 31 and sheathed with a lead alloy coating. The alloy contains 0.05% tellurium and 0.067% copper.

What I claim as my invention and desire to 5 secure by Letters Patent is:—

1. A method of manufacturing an extruded product, which comprises alloying lead with a proportion of from 0.02 to 0.25% of tellurium and from 0.03 to 0.1% of copper, and submitting 10 the alloy to extrusion at temperatures equal to those customarily employed for extruding ordinary soft lead to obtain a product which has a fine grain structure throughout despite the high extrusion temperature. 15

2. A method of manufacturing an extruded product, which comprises alloying lead with a proportion of from 0.02 to 0.25% of tellurium and from 0.06 to 0.07% of copper, and submitting 20 the alloy to extrusion at temperatures equal to those customarily employed for extruding ordinary soft lead to obtain a product which has a fine grain structure throughout despite the high extrusion temperature, and is capable of being locally welded without introducing a coarse 25 structure as a result of fusion.

3. A method of manufacturing an extruded product, which comprises alloying lead with a proportion of from 0.02 to 0.1% of tellurium and from 0.06 to 0.07% of copper, and submitting 30 the alloy to extrusion at temperatures equal to those customarily employed for extruding ordinary soft lead to obtain a product which has a fine grain structure throughout despite the high extrusion temperature, and is capable of being locally welded without introducing a coarse structure as a result of fusion.

4. An extruded product made from an alloy consisting preponderantly of lead and containing from 0.02 to 0.25% of tellurium and from 0.03 to 0.1% of copper, which product has been extruded at temperatures equal to those customarily employed for extruding ordinary soft lead, and has a fine grain structure throughout.

5. An extruded product made from an alloy consisting preponderantly of lead and containing from 0.02 to 0.25% of tellurium and from 0.06 to 0.07% of copper, which product has been extruded at temperatures equal to those customarily employed for extruding ordinary soft lead and has a fine structure throughout, and can be locally welded without introducing a coarse structure as a result of fusion.

6. An extruded product made from an alloy consisting preponderantly of lead and containing from 0.02 to 0.1% of tellurium and from 0.06 to 0.07% of copper, which product has been extruded at temperatures equal to those customarily employed for extruding ordinary soft lead, and has a fine grain structure throughout, and can be locally welded without introducing a coarse structure as a result of fusion.

7. The extrusion at temperatures equal to those customarily employed for the extrusion of ordinary soft lead, of a ternary alloy of lead, tellurium and copper, containing a proportion of tellurium in beneficial amount not exceeding 0.25% and a proportion of from 0.03%-0.1% of copper, whereby an extruded product is obtained having a fine grain structure throughout notwithstanding the high extrusion temperature employed. 70

BRINLEY JONES.